

## UNITED STATES PATENT OFFICE

ERWIN FAHRLÄNDER, OF PFORZHEIM, GERMANY

## SALT BATH FOR ANNEALING METAL ARTICLES

No Drawing. Application filed June 23, 1930, Serial No. 463,373, and in Germany January 30, 1930.

The salt baths, serving for annealing articles made of precious metals and their alloys, should have the following properties:

The melting point should as much as possible not exceed 600° C., in order for example to prevent baking together of the thin silver sheeting, when it is annealed in roll shape.

The bath liquor must further possess good covering power, that is the annealed article must be covered on withdrawal with a thin and at the same time dense protecting layer, so that access of air is excluded on the way to the cooling liquid into which the article 15 annealed is to be dipped, and this article cannot tarnish.

Finally the bath liquor must not act chemically on the articles being annealed, as otherwise discoloring of the surface and the 20 like will occur, which is of great disadvantage, especially in the case of plated articles.

The salt baths hitherto known do not possess these properties, and they cannot 25 be used without disadvantage for annealing articles made of precious metals and of the alloys of the same.

It has definitely been possible, to attain the necessary thin liquidity necessary for annealing such articles by adding cyanide compounds, but the use of cyanide compounds is open to the following objections:

They have a great tendency to decompose, so that the composition of the bath does not 35 remain constant. The temperature of the bath changes with the alteration of the potassium, for example of cyanide content, if the bath has to be maintained at a uniform degree of thin liquidity. Moreover, owing 40 to the presence of cyanide compounds vapors are produced when quenching the articles, which have a great tendency to cause sneezing. There are also difficulties in getting rid of the waste water containing cyanide of potassium.

The salt bath mixtures with a high percentage of common salt are certainly remarkable for their cheapness, but they possess very little or no covering power. If they contain soda or potash, they give for 50 example a greenish color to plated articles.

It has been found, that the discolorings and the other objections to the known salt baths do no longer occur, if to the mixture of common salt and potash, to which larger 55 quantities of potassium sulphate are added, the proportion of soda to the potassium is not greater than 1. If the proportion is inverse, the melting point of the mixture rises 60 in a very short time, that is, if the temperature of the bath is maintained constant, it will quickly become viscous and useless.

Suitable compositions for the bath are:

|                     | Percent |
|---------------------|---------|
| I. Common salt      | 65      |
| Potassium sulphate  | 46      |
| Potassium carbonate | 11      |

For improving the covering power of 70 these baths, sodium phosphate or borax may be added in small quantities up to 6%. The following may be mentioned by way of example as bath compositions containing these constituents.

|                     | Percent |
|---------------------|---------|
| II. Common salt     | 30      |
| Potassium sulphate  | 44      |
| Potassium carbonate | 21      |
| Borax               | 5       |

|                     | Percent |
|---------------------|---------|
| III. Common salt    | 30      |
| Potassium sulphate  | 44      |
| Potassium carbonate | 21      |
| Sodium phosphate    | 5       |

Baths having a very good covering power, which are not affected by the material being annealed and are therefore particularly suitable for plated articles, are obtained from the above mixtures by the admixture 90

of mineral alkaline carbonates or oxides up to 10%. The following are examples:

|                        | Percent |
|------------------------|---------|
| 5 IV. Common salt      | 28      |
| 5 Potassium sulphate   | 41.5    |
| 5 Potassium carbonate  | 21      |
| 5 Borax                | 4.5     |
| 5 Magnesium carbonate  | 2.5     |
| 10 Calcium carbonate   | 2.5     |
| 10 V. Common salt      | 25      |
| 10 Potassium sulphate  | 54      |
| 10 Potassium carbonate | 15      |
| 10 Magnesium carbonate | 3       |
| 15 Calcium carbonate   | 3       |
| 15 VI. Common salt     | 25      |
| 15 Potassium sulphate  | 54      |
| 15 Potassium carbonate | 15      |
| 20 Magnesium oxide     | 3       |
| 20 Calcium oxide       | 3       |

The proportion of pure sodium to pure potassium is in the Examples I to VI: 1: 1.33; 1: 2.55; 1: 2.5; 1: 1.22; 1: 3.2 and 1: 3.2, that is not greater than 1.

25 It may happen, that a bath of this kind becomes black, especially when heated from above, if this is carried out for protecting the crucible, owing to the flame coming directly into contact with the salt mixture.

30 In order to overcome this objection 0.1 to 0.2% of saltpeter may be added to the bath.

The annealing baths are suitable also for many nonprecious metals and alloys.

35 I claim:

1. A salt bath for annealing metal articles, consisting in a mixture of common salt, potash and potassium sulphate, the proportion of the sodium to the potassium being not greater than 1, with addition of mineral alkaline oxides including magnesium to a maximum of 10%.

40 2. A salt bath as specified in claim 1, comprising in admixture 25% common salt, 54% potassium sulphate, 15% potassium carbonate, 3% magnesium oxide and 3% calcium oxide.

45 In testimony whereof I affix my signature.

ERWIN FAHRLÄNDER.